

Sept. 17, 1935.

H. D. MURRAY

2,014,692

FERRO-PRUSSIATE PRINTING

Filed March 3, 1934



## UNITED STATES PATENT OFFICE

2,014,692

## FERRO-PRUSSIATE PRINTING

Humphrey Desmond Murray, South Kensington,  
London, England, assignor of two-thirds to  
Douglas Arthur Spencer, London, England, and  
Norton & Gregory Limited, London, England, a  
British company

Application March 3, 1934, Serial No. 713,944  
In Great Britain March 10, 1933

8 Claims. (Cl. 95—6)

This invention is for improvements in and relating to ferro-prussiate printing, and comprises an improved sensitized base and an improved print and also their process of production.

5 It is well known to prepare a light-sensitive base, usually paper, by coating with a solution containing a ferric salt and a ferricyanide and drying. On exposure of such a base to light behind a design, the ferric salt on the portions un-  
10 screened from the light is reduced to a ferrous salt, which is capable of reacting with the ferricyanide to produce a blue colour. The prints are fixed by washing the base in water, whereby the soluble salts are removed and so further action  
15 of light prevented. This process is commonly known as the ferro-prussiate, or blue-print, process.

Hereinafter, a base which has been treated with light-sensitive reagents in the manner just described will be referred to as a ferro-prussiate paper and a print therefrom as a ferro-prussiate print. The word "paper" is intended to include, as well as paper itself, any other suitable base.

According to this invention, a ferro-prussiate print is produced by treating a ferro-prussiate paper, after exposure, with a fixing agent for one or other of the primary reagents with which the paper has been coated, for the purpose of directly developing the picture to a light-resistant print.

Thus, if the exposed paper be treated, for example, sponged over, with a dilute solution of a weak alkali, such as borax or an alkali perborate, the negative image is fixed in the sense that it may be further exposed to light without turning blue. Orthophenanthroline is an example of another type of compound which, possessing the property of forming a non-reactive co-ordinated compound with iron, may be employed. This method of fixing the residual iron salt has, however, the disadvantages of reducing the colour of the blue background and tending to make the lines of the image run. Substances which fix only the iron salt in the exposed print  
40 do not appear to have the power of preserving the blue background against the bleaching action of light over long exposure, and it is preferred, therefore, to utilize a developer whose primary function is to fix the unchanged ferricyanide; and this developer may comprise an agent having the property of fixing the residual iron salt, as will be presently explained.

According to this preferred form of the invention, the ferro-prussiate paper is treated subsequent to exposure to light with a ferricyanide

insolubilizer or fixing agent, that is to say, an agent capable of reacting with the soluble ferricyanide to give an insoluble derivative. Examples of suitable agents of the kind are, in order of preference, solutions of salts of nickel, zinc, manganese, cadmium and cobalt.

Soluble organic bodies, capable of giving insoluble compounds with ferricyanides, may be employed; but a not uncommon drawback to such reagents is that they frequently impart undesirable colours to the print particularly on exposure to light and air. For example, a ferro-prussiate paper treated with a developing solution containing the basic dyestuff Auramine, Colour Index 655, and a mild oxidizing agent, is rendered stable to exposure to light if the exposure be not too prolonged.

For the most effective results, the ferricyanide insolubilizer should be employed in as high a concentration as is consistent with avoidance of crystallization upon the surface of the print as the developing solution dries. Thus, for application in a thin uniform film by mechanical means, solutions of the following concentrations may be used:

|                    | Per cent |
|--------------------|----------|
| Nickel sulphate    | 15-20    |
| Manganese sulphate | 20-30    |
| Zinc sulphate      | 30-40    |

For application by hand, these solutions should be diluted in the proportion of 3 volumes of water per 10 volumes of solution in order to allow for the greater quantity of liquid received by the paper. Otherwise the salts may crystallize and form a bloom.

The respective colours of the lines produced by the aforesaid metal salt developers are as follows:

|                 |               |
|-----------------|---------------|
| Nickel salts    | Bright yellow |
| Zinc salts      | Pale yellow   |
| Manganese salts | Salmon pink   |
| Cadmium salts   | Pale yellow   |
| Cobalt salts    | Brick red.    |

A diagrammatic illustration of the carrying out of the present invention is given by way of example in the accompanying flow sheet. This flow sheet shows the object, that is the transparency bearing a cross as the design, the unexposed paper, the exposed paper obtained by exposing the paper behind the object, and the various final prints which may be obtained by treating the exposed paper with one of the various salts set out above.

The developing solution may also comprise a

wetting agent, that is, a substance which lowers the surface tension of the solution, thereby increasing the tendency of the liquid to spread and to penetrate into the material of the base.

5 I have found it to be distinctly advantageous that the ferro-prussiate print should comprise an oxidizing agent, which may be conveniently applied as a component of the developing solution. Such an agent appears to fulfill at least two 10 functions; darkening the colour of the background and increasing the stability of the print towards light. My experience has also shown that the best effect is obtained by the association of a strong or quick-acting oxidizing agent, such 15 as a persulphate, with a comparatively mild or slow-acting oxidizer, such as a chlorate. A chlorate may also be used alone.

The stronger oxidizer need only be present in the developing solution in sufficient concentration 20 to bring out the full depth of colour of the background. For example, a suitable concentration for ammonium persulphate is 2 per cent. The slow-acting oxidizer should be employed in the highest possible concentration consistent with 25 avoidance of crystallization. For example, a solution for mechanical application may contain about 10-20 per cent of sodium chlorate.

I have further found that in the development 30 of ferro-prussiate prints with a ferricyanide-insolubilizer it is desirable carefully to adjust the acidity of the base and of the developing solution so that, on the one hand, there shall not be present enough free acid to dissolve any of the insoluble ferricyanide produced and so give rise to free 35 ferricyanide ions capable of causing discolouration in the originally screened parts of the base on re-exposure of the latter to light, and that, on the other hand, the base shall be on the acid side of neutrality in order that the Prussian blue 40 of the background may not be bleached. Mild alkalies have the effect of converting Prussian blue into a white leuco-compound, especially on exposure to air, and hence are not to be recommended by themselves for adjustment of the 45 acidity. Such adjustment is preferably made by applying the ferricyanide-insolubilizer in a buffered solution.

It appears probable that the presence in the 50 developer of a buffer reagent permits of the formation on the prussiate paper of insoluble basic salts of iron in place of the original soluble iron salts with which the paper was coated. This reaction reinforces the effect produced by precipitating an insoluble ferricyanide in place of 55 the soluble ferricyanide originally coated on the paper. If the ferric ion be bound in an insoluble compound at the same time that the ferricyanide ion is bound in an insoluble compound, the chance is reduced of the formation of either ferric ferrocyanide or ferrous ferricyanide—both of 60 which are coloured—when the print is exposed in light.

The buffer mixture should maintain a sufficiently high acidity to permit the full development 65 of the blue colour where the sensitized paper has been initially exposed to light. A suitable buffer reagent is provided by an ammonium or alkali salt of a weak acid, such as an ammonium or alkali acetate or citrate, together with an appropriate acidifier; but the preferred buffer 70 reagent is a mixture of a monobasic and dibasic phosphate in approximately equal proportions with or without a small amount of an acid sulphate.

75 The following are examples of suitable mix-

tures which may be added to the developing solution:

8% of potassium citrate plus 4 per cent of citric acid.

7% of sodium acetate plus 3 per cent of acetic acid.

5% of diammonium hydrogen phosphate plus 5 per cent of ammonium dihydrogen phosphate.

This phosphate mixture has a pH value of about 4.0, and this appears to be the optimum reaction 10 for the developer.

The process is carried out to the best advantage with ferro-prussiate papers which do not contain, as is usually the case, an excess of ferric salt 15 relatively to ferricyanide, because this excess causes a gradual fading of the background in the finished print; but a drawback to the use of such paper is that an excess of ferricyanide relatively to ferric salt results in slow printing, probably because the yellow colour of the ferricyanide inhibits full action of the blue actinic rays upon the salt of iron. An excess of ferricyanide carries also this disadvantage, that, a large concentration of iron salt not being possible, the maximum depth of colour of the paper is not 25 great.

The comparatively small depth of colour of a ferro-prussiate paper of the above type may be corrected in one way by applying to the surface 30 a suitable colouring matter as nearly as possible complementary in colour to Prussian blue. For example, the developer may include a small quantity of a substantially complementary yellow dyestuff, whereby a print may be obtained which shows bright yellow lines upon a dark-green background.

A ferro-prussiate paper as aforesaid, wherein ferricyanide is definitely in excess of ferric salt, may be prepared by first coating or impregnating the base with the ferricyanide and then, after 40 drying, with the ferric salt. A paper so prepared provides, notwithstanding the excess of ferricyanide, a fairly quick-printing medium. Alternatively, the iron and ferricyanide may be applied together, but the former process appears to 45 be the more advantageous.

For the most satisfactory results, especially as regards the stability of the print, it is desirable to use a paper of low content in sulphite-treated pulp; and a good class paper is to be recommended. 50

It is preferred, both for the manufacture of a ferro-prussiate paper and for the development thereof according to this invention, to apply the appropriate reagents to the base by a machine, desirably of that type which provides for the 55 distribution of the reagent in a thin and uniform film over the surface of the base.

#### Example I

A ferro-prussiate paper after exposure to light 60 behind a design was sponged over by hand with a solution containing 10 grams of manganese sulphate in 100 cc. of water, and was then dried.

#### Example II

A ferro-prussiate paper after exposure to light 65 behind a design was fixed in a coating machine carrying a thin film of liquid over the surface of the paper from a trough charged with a solution containing 20 grams of nickel sulphate and 4 70 grams of potassium persulphate dissolved in 100 cc. of water.

#### Example III

A ferro-prussiate paper after exposure to light 75 behind a design was fixed in a machine as in Ex-

ample II by treatment with a solution containing 10 grams of zinc chloride; 2 grams of potassium persulphate and 1 cc. of sulphuric acid dissolved in 100 cc. of water.

5 **Example IV**

A ferro-prussiate paper after exposure to light behind a design was fixed in like manner in a machine by treatment with a developing solution of the composition:

|                               |          |
|-------------------------------|----------|
| Nickel sulphate               | 88 grams |
| Ammonium persulphate          | 13 grams |
| Ammonium dihydrogen phosphate | 22 grams |
| Diammonium hydrogen phosphate | 22 grams |
| 15 Sodium bisulphate          | 6 grams  |
| Sodium chlorate               | 44 grams |
| Water                         | 440 cc.  |

This formula may be varied by replacing the nickel sulphate by a substantially equal weight of zinc or manganese sulphate. If applied by hand, for example, by a sponge, the solution should be diluted in the proportion of 3 parts by volume of additional water to every 10 parts by volume of the solution, as previously explained.

20 **Example V**

A sheet of slightly absorbent, good quality rag-paper was treated in a coating machine with a 30 solution composed of:

|                        |           |
|------------------------|-----------|
| Potassium ferricyanide | 7 ozs.    |
| Water                  | 4,000 cc. |

and then, after drying, was treated in like manner 35 with a solution composed of:

|                         |           |
|-------------------------|-----------|
| Ferric ammonium oxalate | 3.5 ozs.  |
| Ammonium oxalate        | 5 ozs.    |
| Water                   | 4,000 cc. |

40 The paper so prepared, carrying an excess of ferricyanide relatively to the ferric salt, was exposed to light behind a design and the print developed in a developing machine with a solution of the following composition:

|                                |          |
|--------------------------------|----------|
| Nickel sulphate                | 20 grams |
| Ammonium persulphate           | 2 grams  |
| Potassium dihydrogen phosphate | 5 grams  |
| Disodium hydrogen phosphate    | 5 grams  |
| 50 Sodium bisulphate           | 2 grams  |
| Water                          | 100 cc.  |

Alternatively, the above quantity of ferricyanide (7 ozs.) may be dissolved in the ferric ammonium oxalate solution, and the paper then 55 coated with this latter.

The invention eliminates the washing procedure of the usual ferro-prussiate process and provides a rapid and easy method of positive development of ferro-prussiate papers with production of an 60 improved picture; and also permits of the conjoined use of a printing and a developing machine, so that finished prints may be made from a plan with increased facility and speed of operation.

65 I claim:

1. A process for the production of stable photographic prints consisting in exposing to light a layer of light sensitive material containing a soluble ferric salt and a soluble ferricyanide behind a transparency, and surface treating the exposed layer with an aqueous solution containing a chemical fixing agent for one of the primary reagents of the layer in order to effect a chemical transformation of the primary reagent present in the unexposed parts of the layer and so render the 70

unexposed parts of the layer non-sensitive to light.

2. A process for the production of stable photographic prints consisting in exposing to light a 5 layer of light sensitive material containing a soluble ferric salt and a soluble ferricyanide behind a transparency, and surface treating the exposed layer with an aqueous solution containing a salt of one of the metals of the group consisting of nickel, cadmium, manganese, zinc and cobalt, 10 in order to effect a chemical transformation of the ferricyanide present in the unexposed parts of the layer and so render the unexposed parts of the layer non-sensitive to light.

3. A process for the production of stable photographic prints consisting in exposing to light a 15 layer of light sensitive material containing a soluble ferric salt and a soluble ferricyanide behind a transparency, and surface treating the exposed layer with an aqueous solution containing a weak 20 alkali in order to effect a chemical transformation of the ferric salt in the unexposed parts of the layer and so render the unexposed parts of the layer non-sensitive to light.

4. A process for the production of stable photographic prints consisting in exposing to light a 25 layer of light sensitive material containing a soluble ferric salt and a soluble ferricyanide behind a transparency, and surface treating the exposed layer with an aqueous solution containing ortho- 30 phenanthroline in order to effect a chemical transformation of the ferric salt in the unexposed parts of the layer and so render the unexposed parts of the layer non-sensitive to light.

5. A process for the production of stable photographic prints consisting in exposing to light a 35 layer of light sensitive material containing a soluble ferric salt and a soluble ferricyanide behind a transparency, and surface treating the exposed layer with an aqueous solution containing a 40 chemical fixing agent for one of the primary reagents of the layer and an oxidizing agent in order to effect a chemical transformation of the primary reagent present in the unexposed parts of the layer and so render the unexposed parts of the 45 layer non-sensitive to light.

6. A process for the production of stable photographic prints consisting in exposing to light a 50 layer of light sensitive material containing a soluble ferric salt and a soluble ferricyanide behind a transparency, and surface treating the exposed layer with an aqueous solution containing a chemical fixing agent for one of the primary reagents of the layer and both a strong and a mild 55 oxidizing agent in order to effect a chemical transformation of the primary reagent present in the unexposed parts of the layer and so render the unexposed parts of the layer non-sensitive to light.

7. A process for the production of stable photographic prints consisting in exposing to light a 60 layer of light sensitive material containing a soluble ferric salt and a soluble ferricyanide behind a transparency, and surface treating the exposed layer with an aqueous solution containing a 65 chemical fixing agent for one of the primary reagents of the layer and a buffer reagent in order to effect a chemical transformation of the primary reagent present in the unexposed parts of the layer and so render the unexposed parts of the 70 layer non-sensitive to light.

8. A process for the production of stable photographic prints consisting in preparing a ferro-prussiate paper by applying a solution of ferricyanide to the paper, permitting the solution to 75

dry, and then applying a solution of ferric salt in such a quantity that an excess of ferricyanide over ferric salt is obtained on the paper, exposing the ferro-prussiate so obtained to light behind a transparency, and surface treating the exposed layer with an aqueous solution containing a chemical fixing agent for one of the primary re-

agents of the layer in order to effect a chemical transformation of the primary reagent present in the unexposed parts of the layer and so render the unexposed parts of the layer non-sensitive to light.

HUMPHREY DESMOND MURRAY.